

# UNITED STATES PATENT OFFICE.

GEORGE J. GREGERSON, OF NEW YORK, ASSIGNOR OF ONE-HALF OF HIS  
RIGHT TO EMMA L. HAYWARD, OF PORT RICHMOND, N. Y.

## PROCESS OF TREATING PINE-LEAVES AND OTHER VEGETABLE FIBERS.

SPECIFICATION forming part of Letters Patent No. 229,248, dated June 29, 1880.

Application filed February 27, 1880.

*To all whom it may concern:*

Be it known that I, GEORGE J. GREGERSON, of the city, county, and State of New York, have invented a new and useful Process 5 of Treating Pine-Leaves and other Vegetable Fibers, of which the following is a specification.

This invention relates to a new method of treating the fiber such as contained in pine-leaves or other analogous fibrous substances, either in their natural or in their dry state, so 10 as to separate the fibrous matter from the foreign substances found associated therewith, and thereby obtaining a pulpy mass suitable 15 for manufacture of paper, or a fibrous mass for other uses in the arts.

The following are the steps when the material to be treated is in its natural state and in order to obtain the fiber in a pulpy condition: 20 First, extracting the essential oils, in order to prepare the mass for fermentation; second, fermentation, in order to put the mass in a condition for freeing it from resinous matter; &c.; third, the carrying off of the resinous 25 matter, &c., and for softening the fiber and bringing it into an elastic state; fourth, freeing the mass from alkaline matter—that is to say, bringing such matter into salts, while at same time disintegrating the mass, and then 30 washing out the salts.

I therefore, to obtain such product, proceed as follows:

First. I place the vegetable matter—such, for instance, as fine leaves—in a large tank. 35 This tank is constructed with a false bottom, situated about six inches above its true bottom, the false bottom being perforated. A pipe is so arranged as to supply steam between these two bottoms. The cover to the 40 tank is made to fit it closely, and there is connected to the center of such cover a pipe leading off into a reservoir at the side of the tank. The tank is not quite filled up to the top with leaves, a few inches' space being left, and the 45 material is saturated with either cold or warm water introduced at the top of the tank. In order to hasten the operation, the leaves or other material may be cut before being placed in the tank. The cover being placed on the 50 tank, steam is then introduced between the

two bottoms and the heat carried up from about 150° to 180° Fahrenheit. The vapor which will now arise in the space between the material and the cover will be carried off through the pipe in the cover, and pass 55 into the reservoir, and be there condensed, thereby producing essential oils, which production, however, is no part of this present process. This evaporation is continued until the material is deprived of the essential oils 60 contained therein, and then the liquor contained in the tank is drawn off by means of a faucet located between the false and true bottom.

The material is now ready to be treated by 65 the next step, as follows:

Second: I now put the material, as above treated, in an apparatus known as a "vinegar-generator." Then a liquor is made out of the liquor drawn off at the end of the first step of 70 the operation, to which is added alcohol in the proportion of about one gallon of alcohol to ten gallons of the liquor. Such new liquor is then poured over the material in the generator and drawn off through a faucet in the 75 lower portion of the generator. This operation is continued from time to time for the purpose of creating fermentation. The temperature of the mass is kept up to about 75° or 80° Fahrenheit. The contact of the air with the 80 minutely-divided liquid promotes the operation, which consists essentially in the oxidation of the alcohol. When the fermentation is complete, the material is in a softened condition and ready to be transferred to the proper 85 apparatus for the third step of the operation.

Third. The mass is now placed in an iron tank of proper size to hold any large or given mass to be treated, the shape or form not being essential, so long as it is strong enough to 90 withstand the required pressure. I prefer at this step to use a kier, such as employed in the ordinary bleaching process. When the kier is filled the man-hole is closed. Steam is then let into the kier and the pressure carried 95 up to the required degree. The heat dissolves the resinous and analogous substances contained in the material, and they are discharged through a faucet at the lower end of the kier into a reservoir placed near that point. The 100

degree to which the pressure is carried depends upon the fibrous material being treated and the character of product to be produced. When pine-leaves are treated, which contain 5 in their composition a large amount of fiber and resinous material, a high pressure is required to take out the woody and resinous materials and to make the resulting fiber soft and elastic. I therefore employ therewith a range 10 of pressure from 200° to 500° Fahrenheit. When other leaves or material of more delicate texture are treated, and also with fine leaves, when a less soft and elastic product is required, a pressure varying between 25° and 15 200° may be used with excellent results. A high pressure is necessary to obtain a very soft fiber, such as to produce a pulp for manufacturing paper out of, or for use in the manufacture of cloth, felt, &c. The duration of time 20 of the treatment with steam is from six to ten hours. I do not, therefore, confine myself to any degree of heat or duration of time for treating the material at this stage, so long as fiber is separated from the other material, as 25 it can be used for some purpose or other treated at any degree of heat above 25°, its degree of hardness or softness after being so separated by heat and pressure determining its fitness for some one use or the other in the arts.

30 Fourth. I now treat the fiber so separated and properly softened with a diluted acid—either sulphuric, muriatic, or equivalent acid—for the purpose of converting the vegetable alkali remaining in the fiber into salts, which 35 is done in a "hollender," so called, and at same time the fiber thus becomes disintegrated more or less, depending upon the time it is left in the vessel. The salts may then be washed out of the mass by clean water, and a pulpy mass 40 of fiber is left in a more or less soft condition. The product may be subsequently bleached, if desired, for any particular use in the arts.

When the material is in a dry state, to obtain a pulpy mass, the first step of the process may be omitted, as there are no essential oils 45 to be got rid of. The operation may be commenced at the second step—that is, with the creation of fermentation in the mass.

When it is desired to obtain a fibrous mass, such as required for use in mattresses, cushions, and other upholstery purposes, the first 50 and second steps are both dispensed with, whether the fibrous material treated is in its natural or in its dry state.

I claim—

1. The process of treating vegetable fiber by first extracting the essential oils, and then freeing the mass from resinous matter by means of fermentation and by heat and pressure, and then from the alkaline matter by a 60 subsequent treatment as will reduce such alkaline matter into salts, and then washing out such salts, substantially as described.

2. The process of treating vegetable fiber by freeing the mass from resinous matter by 65 means of fermentation and by heat and pressure, and then from the alkaline matter by a subsequent treatment as will reduce such alkaline matter into salts, and then washing out such salts, substantially as described.

3. The process of treating vegetable fiber by freeing the mass from resinous matter by means of heat and pressure, and then from the alkaline matter by a subsequent treatment as will reduce such alkaline matter into salts, 75 and then washing out such salts, substantially as described.

GEORGE J. GREGERSON.

Witnesses:

JAMES H. HUNTER,  
ANDREW M. TODD.

55

50

70

75